

# United States Patent Office

2,822,267

Patented Feb. 4, 1958

1

2,822,267

## MAGNESIUM ALLOY

George S. Foerster, Midland, Mich., assignor to The Dow Chemical Company, Midland, Mich., a corporation of Delaware

No Drawing. Application November 18, 1955  
Serial No. 547,821

4 Claims. (Cl. 75—168)

The invention relates to magnesium-base alloys. It more particularly concerns an improved magnesium-base alloy containing thorium, zinc, and zirconium.

Attempts to produce magnesium-base alloys containing thorium, zinc, and zirconium have not met with much commercial success due at least in part to the high thorium content heretofore proposed which makes the alloys excessively costly without achieving the most desirable combination of mechanical properties. It has now been discovered that by compounding the magnesium-base alloy of small amounts of the alloying metals thorium, zinc, zirconium, and rare earth metal an exceptional combination of extreme lightness, high strength, high resistance to corrosion and other desirable properties is obtained. The invention then consists of the improved magnesium-base alloy herein described and particularly pointed out in the claims.

In compounding the alloy, there is melted together enough of the alloying metals to provide an alloy containing in parts by weight, from 0.2 to 1.2 percent of zinc, 0.4 to 0.8 percent of zirconium, and from 0.1 to 0.75 percent of thorium, 0.1 to 1 percent of rare earth metal, and magnesium in amount sufficient to make up the balance. From the foregoing proportions of the metals in the alloy, it is manifest that the alloy contains at least about 96.45 percent of magnesium except for the small amounts of impurities normally present in commercial magnesium, say 0.1 to 0.3 percent by weight, when the alloy contains the maximum amounts of the other metals. Similarly, the maximum amount of magnesium which is present when the other metals are present in their smallest proportions is 99.2 percent. Because of the relatively high magnesium content of the alloy, it possesses substantially the same lightness characteristic of

2

Melting may be done in a suitable crucible with the protection from atmospheric attack of a covering of a saline flux free from magnesium chloride. A saline flux composed of 57 parts of KCl, 28 parts of CaCl<sub>2</sub>, 12.5 parts of BaCl<sub>2</sub>, and 2.5 parts of CaF<sub>2</sub> by weight is suitable for use in the melting and alloying operation. After the metals are melted together, the resulting alloy may be refined by stirring the molten alloy with additional saline flux. The so-refined alloy is allowed to settle and after settling is separated from the flux as by decantation and run into a suitable casting mold, e. g. a slab mold for rolling stock or an ingot mold for extrusion.

A preferred range of proportions of the alloying metals is: zinc 0.5 to 1 percent, zirconium 0.5 to 0.7 percent, thorium 0.3 to 0.7 percent, and rare earth metal 0.4 to 0.8 percent, e. g. misch metal. A desirable specific alloy formulation within the scope of the invention is one having 0.5 percent of thorium, 0.8 percent of zinc, 0.6 percent zirconium, the balance being magnesium.

In sheet form, as produced by rolling a cast slab of the alloy, the alloy possesses static tensile properties at 70°-600° F. at least as good as, and in many cases better than, any magnesium-base sheet alloy heretofore known containing thorium, zinc, and zirconium but without the high thorium content of conventional magnesium-base alloys. Its secondary properties, such as formability, toughness, rollability, weldability, and corrosion resistance, are superior to any known magnesium-base alloy containing larger amounts of thorium, zinc, zirconium, and rare earth metal. For example, the corrosion resistance as measured by the weight loss in the conventional alternate immersion test in 3 percent aqueous sodium chloride solution at 95° F. for 14 days is at least as good as high purity magnesium, i. e. the weight loss is not greater than about 0.2 milligram per square centimeter per day in the said test. The trace of attack which occurs during the corrosion rate test in 14 days is quite uniformly distributed over the surface of the metal.

Alloys within the scope of the invention having a zinc content of 0.2 to 0.7 are cold-rollable to foil thickness, e. g. 0.003 inch from sheet 0.125 inch thick, without an intermediate anneal.

The alloys of the invention find their greatest usefulness in applications requiring high strength both at room temperature as well as moderately elevated temperature, e. g. up to 600° F.

The following examples which are set forth in the accompanying table are illustrative of the invention.

| Alloy No. | Properties 1 |            |            |            |           |        |     |    |           |         |    |           |         |    |  |
|-----------|--------------|------------|------------|------------|-----------|--------|-----|----|-----------|---------|----|-----------|---------|----|--|
|           | Composition  |            |            |            |           | 70° F. |     |    |           | 400° F. |    |           | 600° F. |    |  |
|           | Percent Zn   | Percent Zr | Percent RE | Percent Th | Percent E | TYS    | CYS | TS | Percent E | TYS     | TS | Percent E | TYS     | TS |  |
| 1-----    | 0.5          | 0.6        | 0.5        | 0.3        | 4         | 37     | 35  | 44 | 10        | 27      | 29 | 42        | 14      | 16 |  |
| 2-----    | 1.0          | 0.6        | 1.0        | 0.5        | 5         | 37     | 36  | 45 | 15        | 27      | 30 | 50        | 13      | 15 |  |
| 3-----    | 1.0          | 0.6        | 0.5        | 0.5        | 6         | 36     | 36  | 44 | 22        | 24      | 28 | 64        | 13      | 13 |  |
| 4-----    | 0.5          | 0.6        | 0.5        | 0.5        | 6         | 36     | 34  | 42 | 14        | 25      | 28 | 48        | 13      | 13 |  |

<sup>1</sup> Strength given in nearest 1,000 lbs. per square inch of rolled test specimens.  
TYS=Tensile yield strength at 0.2 percent deviation from the modulus line.  
CYS=Compression yield at 0.2 percent deviation from the modulus line.  
TS=Ultimate tensile strength.  
E=Elongation.

magnesium but enhanced mechanical properties, thereby making the alloy useful for many structural purposes.

The rare earth metals suitable for use in the invention are: Ce, La, Pr, Nd, or misch metal. Misch metal with from 35 to 80 percent of cerium, the balance being other rare earth metal and up to 5 percent of non-rare earth metal, is the preferred rare metal ingredient of the alloy. Any of the foregoing rare metals may be used alone or in any combination in compounding the alloy.

The alloy of the invention is readily rolled hot from any thickness of suitable rolling stock to desired gauge. In preparing the alloy for rolling the melt of the desired alloy may be cast into slabs. The cast slabs are then scalped to remove the surface skin in which impurities usually collect. The scalped slabs may then be heat treated, as by soaking at 800°-850° F. for 8 hours. Hot rolling is commercial at 800° to 850° F. and when the temperature of the metal falls to between about 650° and

700° F. the rolled metal, if not reduced to the desired gauge, is reheated to 800°-850° F. and rolled again. This procedure is repeated until the desired thickness is obtained. Following hot rolling, the rolled metal may be annealed at 800°-850° F. and then cold rolled at 1 to 2 percent reduction in thickness per pass to as much as 40 percent total thickness reduction at room temperature. A final anneal may be given after cold rolling depending upon the temper desired. A hard temper is obtained by heating for 1 hour at 500° F. a soft temper by heating for 1 hour at 800° F.

Since zirconium is somewhat difficult to alloy with magnesium, instead of using zirconium itself, it is preferable to use as a source of the zirconium a zirconium rich magnesium-zirconium alloy in making the alloy of the invention. Zirconium which is effectively alloyed with the metals in the alloy is that which will dissolve in hydrochloric acid on subjecting a specimen of the alloy to the dissolving action of the acid. Unalloyed zirconium remains undissolved in this test.

I claim:

1. A magnesium-base alloy consisting of 0.2 to 1.2 percent of zinc, 0.4 to 0.8 percent of zirconium, 0.1 to 0.75 percent of thorium, 0.1 to 1 percent of rare earth metal selected from the group consisting of cerium, lanthanum, praseodymium, neodymium, and misch metal, the balance being magnesium, the zirconium in the said

5

10

15

20

25

alloy being soluble in hydrochloric acid on subjecting the alloy to the dissolving action of the acid.

2. An alloy according to claim 1 in which the rare earth metal is misch metal comprising 35 to 80 percent of cerium.

3. A magnesium-base alloy containing 0.5 to 1 percent of zinc, 0.5 to 0.7 percent of zirconium, 0.3 to 0.7 percent of thorium, and 0.4 to 0.8 percent of misch metal, the balance being magnesium, the zirconium in the said alloy being soluble in hydrochloric acid on subjecting the alloy to the dissolving action of the acid.

4. A magnesium-base alloy containing about 0.8 percent of zinc, 0.6 percent of zirconium, 0.5 percent of thorium, 0.6 percent of misch metal, the balance being magnesium, the zirconium in said alloy being soluble in hydrochloric acid on subjecting the alloy to the dissolving action of hydrochloric acid.

References Cited in the file of this patent

UNITED STATES PATENTS

2,604,396 Jessup ----- July 22, 1952  
2,703,753 Nelson ----- Mar. 8, 1955

OTHER REFERENCES

Ser. No. 369,749, Sauerwald (A. P. C.), published June 16, 1943.